

1

2,920,944

**NON-STALLING GASOLINE FUEL COMPOSITIONS**

Troy L. Cantrell, Drexel Hill, Pa., and John G. Peters, Audubon, N.J., assignors to Gulf Oil Corporation, Pittsburgh, Pa., a corporation of Pennsylvania

No Drawing. Application March 3, 1955  
Serial No. 492,024

3 Claims. (Cl. 44—63)

This invention relates to non-stalling gasoline fuel compositions that are adapted to improve the operation of internal combustion engines under cool, humid atmospheric conditions. More particularly, the invention relates to gasoline fuel compositions that contain a small amount, sufficient to reduce the tendencies of the composition to promote engine stalling in an internal combustion engine of the spark ignition, reciprocating type, of a salt of morpholine and oleic acid.

When an internal combustion engine is operated under cool, humid atmospheric conditions, using a gasoline fuel having a relatively low 50 percent ASTM distillation point, i.e., below about 235° F., excessive engine stalling is apt to be encountered at idling speeds during the warm-up period, especially where engine idling occurs following a period of light load operation. Engine stalling under such conditions has been attributed to the partial or complete blocking of the narrow air passage that exists between the carburetor throat and the carburetor throttle valve during engine idling, by ice particles and/or solid hydrocarbon hydrates that deposit upon and adhere to the metal surfaces of the carburetor parts. Such icing of carburetor parts occurs as a result of the condensation of moisture from the air drawn into the carburetor and as a result of the solidification of such condensed moisture. The aforesaid condensation and solidification of moisture are caused by the refrigerating effect of rapidly evaporating gasoline. Accordingly, excessive engine stalling due to carburetor icing occurs as a practical matter only in the instance of gasolines containing a large proportion of relatively highly volatile components. In practice, a high degree of engine stalling due to carburetor icing has been found to occur, under cool, humid atmospheric conditions, in connection with gasolines having a 50 percent ASTM distillation point below about 235° F.

Excessive engine stalling is, of course, a source of annoyance owing to the resulting increased fuel consumption, battery wear and inconvenience of frequent restarting. It is therefore important that the inherent engine stalling characteristics of gasoline fuels be reduced substantially, where the 50 percent ASTM distillation point of such gasoline fuels is sufficiently low to cause a problem in this respect.

We have found that the stalling characteristics of gasoline fuel compositions that normally tend to promote engine stalling due to carburetor icing are markedly improved by the incorporation therein of a minor amount of a salt of morpholine and oleic acid. In one embodiment of the invention the gasoline composition can also contain about 0.25 to about 0.75 percent by volume of the composition of a light lubricating oil having a viscosity at 100° F. of about 50 to about 500 Saybolt Universal seconds.

The anti-stalling agent included by this invention is a polar, surface active material possessing both hydrophilic and lipophilic properties. While the invention is not limited to any theory of operation, it appears that

2

by virtue of its polarity the morpholine oleate of this invention tends to orient itself upon the metal surfaces of the throttle valve and other critical carburetor parts contacted by the gasoline composition, thus forming a moisture-displacing, residual coating on said carburetor parts, which coating tends to prevent the adherence to said metal surfaces of accumulations of ice of magnitudes sufficient to block the narrow air passages that exist in carburetors at engine idling conditions. It is also considered that the morpholine salts of this invention may orient themselves about small individual water or ice particles, thus tending to prevent the formation of macro-crystals of ice of a size sufficient to block carburetor air passages at engine idling conditions.

When morpholine oleate is utilized in gasoline compositions that contain a small amount of a light lubricating oil the morpholine oleate, by virtue of its affinity for the lubricating oil, tends to attract the oil to the same critical carburetor surfaces referred to above and simultaneously to increase the spreading and metal wetting characteristics of the oil, thus promoting the formation of an adherent oil film on the metal surfaces of the carburetor parts. The oil film thus appears to function in similarly as the morpholine salt itself, but the superior metal wetting properties imparted to the oil by the additive are believed to enable the oil to displace moisture from the metal carburetor surfaces that it would not thoroughly displace alone.

As indicated briefly above, the material which is suitable for addition to gasoline fuel compositions in accordance with the principles of this invention is the addition salt of morpholine and oleic acid.

Morpholine oleate is useful when incorporated in gasoline compositions of the type disclosed in amounts sufficient to reduce the engine stalling characteristics thereof. For example, good results can be obtained with amounts of about 0.001 to about 0.1 percent by weight of the gasoline composition. In most instances a major reduction in the stalling characteristics of gasoline compositions of the type disclosed herein will be obtained by the use of morpholine oleate in amounts of at least about 0.005 percent by weight of the composition. As a practical matter excellent results have been obtained by the use in gasoline of morpholine oleate in amounts not exceeding about 0.01 percent by weight of the composition. Thus, the preferred concentration range according to this invention is about 0.005 to about 0.01 percent by weight of the composition. In order to obtain further improved anti-stalling benefits with very small morpholine salt concentrations, it is sometimes desirable that a small amount of light lubricating oil of the type disclosed be used in conjunction with the morpholine salt.

With respect to the particular concentration ranges mentioned above, it will be appreciated that the optimum concentration of the morpholine salt can vary according to the severity of the atmospheric conditions encountered in the area in which the gasoline is used. With regard to this factor, the problem of engine stalling due to carburetor icing resulting from the refrigeration by evaporating gasoline of moisture condensed from the atmosphere has been observed to be significant at atmospheric temperatures of between about 30° and 60° F., e.g., 35°, 40°, 45°, 50° F., and when the relative humidity is in excess of about 65 percent, e.g., 75, 85, 95, 99 percent. The optimum concentration of anti-stalling additive should be sufficient to effect a substantial reduction in the stalling tendencies of the fuel at the atmospheric conditions of temperature and humidity which are likely to be encountered in service.

In addition to the foregoing factors, the optimum concentration of the anti-stalling additive material varies

principally according to the particular gasoline employed, since the problem of engine stalling is a function of the 50 percent ASTM distillation point of the gasoline fuel. Greater concentrations of the additive combination are normally desirable with decreasing 50 percent distillation points.

Practically speaking, the problem of engine stalling due to carburetor icing caused by rapid evaporation of gasoline occurs only in connection with gasolines having a 50 percent ASTM distillation point of not greater than about 235° F. Accordingly, this invention relates only to gasolines of this type. While occasional engine stalling may occur as a result of carburetor icing at severe atmospheric conditions of temperature and humidity with gasolines having somewhat higher 50 percent ASTM distillation points, experience has indicated that the problem does not assume major importance except with gasolines of the character indicated. The problem of engine stalling due to carburetor icing is especially severe in connection with gasolines having a 50 percent ASTM distillation point of less than about 220° F. The invention is particularly useful in connection with such gasolines. The term "gasoline" is used herein in its conventional sense to include hydrocarbon mixtures having a 90 percent ASTM distillation point of not more than about 392° F. and a 10 percent ASTM distillation point of not more than about 140°.

As previously indicated, the gasoline compositions of this invention are additionally benefited with respect to non-stalling characteristics by the inclusion therein of a small amount of a lubricating oil having a viscosity at 100° F. of between about 50 and about 500 Saybolt Universal seconds; for example, an oil having a viscosity of about 100 S.U.S./100° F. can be used with advantage. Although highly paraffinic lubricating distillates can be used, lubricating distillates obtained from Coastal or naphthenic type crude petroleum oils are preferred because of their superior solvent properties. The lubricating oils utilized in the gasoline compositions of this invention can have been solvent-treated, acid-treated or otherwise refined prior to incorporation into the gasoline compositions of this invention. The lubricating distillates referred to are useful in the gasoline compositions of this invention in amounts of from about 0.25 to about 0.75 percent by volume of the composition, for example 0.5 volume percent. Greater amounts of the lubricating oil can be used but without appreciable further improvement in the stalling tendencies of the gasoline composition; however, the amount of lubricating oil used should not be so great as to adversely affect the solubility and combustion characteristics of the ultimate gasoline compositions.

The morpholine oleate can be incorporated into the base gasoline fuel compositions in any suitable manner. Thus the oleate can be added as such or in the form of dispersions or solutions in solvent such as butanol, isopropanol, ethanol, methanol, 2-butoxyethanol, diethylene glycol monobutyl ether, benzene, toluene, heptane, kerosene, gasoline, mineral oil or the like, which solvents may or may not themselves additionally contribute to the anti-stalling characteristics of the ultimate composition. In some instances it may even be convenient to form the morpholine oleate in situ in the gasoline composition. If desired, the morpholine oleate can be incorporated in gasoline fuel compositions in admixture with other materials designed to improve one or more properties of the gasoline, such as antioxidants, anti-knock agents, ignition control additives, dehazing agents, corrosion inhibitors, dyes and the like.

Gasoline compositions of this invention are further illustrated by the following representative specific examples.

#### EXAMPLE I

An anti-stalling concentrate was prepared by dissolv-

ing 1 percent by weight of morpholine oleate in 99 percent by weight of an aviation grade gasoline described below in greater detail. The foregoing concentrate was incorporated in an aviation grade gasoline that had a 5 strong tendency to promote engine stalling in an amount of 1 percent by weight of the over-all composition. The resulting gasoline composition therefore contained morpholine oleate in a concentration of 0.01 percent by weight of the composition. A typical sample of the base gasoline employed in this example had the following inspections:

|                                       |        |
|---------------------------------------|--------|
| Gravity, ° API                        | 68.0   |
| Sp. gr. 60°/60° F.                    | 0.709  |
| Knock rating                          |        |
| Motor method, octane No.              | 81.6   |
| Aviation lean mixture No., octane No. | 80.2   |
| Aviation rich mixture No., octane No. | 87.5   |
| TEL, ml./gal.                         | 0.49   |
| Heat of combustion, B.t.u./lb. (net)  | 19,020 |
| 20 Vapor pressure, Reid, lb.          | 6.8    |
| Distillation, gasoline                |        |
| Over point, ° F.                      | 122    |
| End point, ° F.                       | 290    |
| 25 10% evap. at ° F.                  | 145    |
| 40% evap. at ° F.                     | 172    |
| 50% evap. at ° F.                     | 180    |
| 90% evap. at ° F.                     | 220    |

#### EXAMPLE II

30 An additional gasoline composition in accordance with this invention and having reduced engine stalling characteristics is prepared by admixture of 1 percent of the anti-stalling concentrate of Example I with the same base gasoline described in Example I, to which there has been 35 previously added 0.5 percent by volume of an approximately 100 S.U.S./100° F. Texas lubricating distillate, a typical sample of which had the following inspections:

|                                                     |       |
|-----------------------------------------------------|-------|
| 40 Gravity, ° API                                   | 24.5  |
| Lbs./gal., 60° F.                                   | 7.55  |
| Viscosity, SUV, sec.:                               |       |
| 70° F.                                              | 235   |
| 100° F.                                             | 106.0 |
| 130° F.                                             | 63.9  |
| 210° F.                                             | 38.3  |
| Viscosity index                                     | 16    |
| Flash, P-M, ° F.                                    | 315   |
| Flash, O.C., ° F.                                   | 320   |
| Fire, O.C., ° F.                                    | 355   |
| Pour, ° F.                                          | 60    |
| Color, ASTM Union                                   | 2.0   |
| Carbon residue, Conradson, percent                  | 0.02  |
| 55 Copper strip test, 212° F. 3 hr.                 | 0     |
| Neutralization value, ASTM D-974-51T—Total acid No. | 0.05  |

60 As heretofore indicated, morpholine oleate produces an appreciable improvement in the stalling characteristics of gasolines that normally tend to promote engine stalling due to carburetor icing. To illustrate the nature of the improvement obtained, in the table following there are presented illustrative results obtained with engine tests using gasoline fuel compositions prepared in accordance with this invention. In order to demonstrate more fully the unusual effectiveness of the morpholine salt of this invention, there are also presented in the following table the results obtained with engine tests of gasoline fuel compositions containing other amine salts.

65 According to the test procedure followed, the fuel compositions to be tested were fed to a standard 216 cubic inch, six cylinder, overhead valve, Chevrolet engine, drawing air through a bed of approximately 2 inch chunks (initial size) of cracked ice packed in a standard ASTM-CFR ice tower. The engine was equipped with a standard Carter Model W-1 carburetor having a

standard Power Glide type throttle damper. The carburetor and fuel system were insulated from the engine by means of a  $\frac{1}{4}$  inch thick asbestos cement board shield, 10 inches in width, which extended the length of the manifold.

The conditions at which the engine was operated are set forth below:

Cooling water temperature, ° F.—

In ----- 75-80  
Out ----- 90-95

Crankcase oil temperature, ° F. ----- 140-150

Carburetor air intake temperature ----- 39-41

Relative humidity, percent ----- 82-85

The operating cycle of the engine included, after temperatures became stabilized, operation for five minutes at 1500 r.p.m. at 5 brake horsepower (B.H.P.) load. During this period the carburetor throttle plate becomes chilled and ice formations are allowed to build up. After this five-minute run, the throttle was closed to the preset position to allow 450 r.p.m. idle speed. If the engine idled satisfactorily for 30 seconds the fuel was considered non-stalling during that operating cycle.

agents and the like can be added to the gasoline compositions of this invention, and the invention specifically includes gasoline compositions containing such additives.

Numerous additional embodiments of the invention will readily suggest themselves to those skilled in the art. 5 Accordingly, we do not intend to be limited by the foregoing description, but rather only by the terms of the claims appended hereto.

We claim:

- 10 1. A gasoline motor fuel composition comprising a major amount of a hydrocarbon mixture boiling in the gasoline range, having a 50 percent ASTM distillation point of less than 220° F., and tending to promote stalling of internal combustion engines, and a minor amount, sufficient to reduce the stalling tendencies of the composition, of a salt of morpholine and oleic acid.
- 15 2. The composition of claim 1 wherein the hydrocarbon mixture contains additionally about 0.25 to about 0.75 percent by volume of the composition of a light lubricating oil having a viscosity at 100° F. of about 50 to about 500 Saybolt Universal seconds.
- 20 3. A gasoline motor fuel composition comprising a major amount of a hydrocarbon mixture boiling in the

Table

| Composition | Base Fuel                                                                 | Additive                                              | Concentration, Active Ingredient, Percent by Wt. | Engine Test: Stalls per 5 Operating Cycles |
|-------------|---------------------------------------------------------------------------|-------------------------------------------------------|--------------------------------------------------|--------------------------------------------|
| 1-----      | Base Gasoline, 180° F. 50% ASTM Distillation Point (Example 1 Base Fuel). |                                                       |                                                  | 5                                          |
| 2-----      | Base Gasoline-----                                                        | Morpholine Oleate of Example 1.                       | 0.01                                             | 0                                          |
| 3-----      | Base Gasoline plus 0.5 Vol. Percent 100 Texas Oil.                        | Triethanol Amine Oleate <sup>1</sup> -----            | 0.01                                             | 5                                          |
| 4-----      | Base Gasoline-----                                                        | Oleates of tert.-C <sub>11-15</sub> Alkyl Amines----- | 0.01                                             | 5                                          |
| 5-----      | "do-----                                                                  | "Tallow"-alkylaminopropylamine Monooleate-----        | 0.01                                             | 5                                          |
| 6-----      | "do-----                                                                  | "Tallow"-alkylaminopropylamine Dioleate-----          | 0.01                                             | 5                                          |

<sup>1</sup> Added to gasoline in form of concentrate consisting of 1 percent solution in mixture of equal volumes of toluene and isopropanol. Gasoline itself failed to dissolve 1 percent triethanol amine oleate.

From the results presented in the foregoing table it will be seen that uninhibited gasolines having a 50 percent ASTM distillation point of less than 235° F. possess poor stalling characteristics, and that such gasolines are markedly improved by incorporation therein of small amounts of morpholine oleate. Thus, comparison of the results obtained with compositions 1 and 2 demonstrates the reduction in stalling characteristics obtained by the invention. Comparison of the results obtained with compositions 2, 3, 4, 5 and 6 demonstrates the marked superiority of morpholine oleate.

To the gasoline fuel compositions of the present invention there can be added one or more additional additive agents designed to improve one or more characteristics of the gasoline fuel. For example, antioxidants, anti-knock agents, ignition control additives, other de-icing agents, anti-rust agents, dyes, lead scavenging

gasoline range, having a 50 percent ASTM distillation point of less than 220° F., and tending to promote stalling of internal combustion engines, and a minor amount, sufficient to reduce the stalling tendencies of the composition, of morpholine oleate, said minor amount being about 0.005 to about 0.01 percent by weight of the composition.

References Cited in the file of this patent

UNITED STATES PATENTS

- 50 2,403,619 Skinner ----- July 9, 1946  
2,466,632 Borus ----- Apr. 5, 1949  
2,600,113 Jones et al. ----- June 10, 1952  
2,667,408 Kleinholtz ----- Jan. 26, 1954  
55 2,668,522 Hickok et al. ----- Feb. 9, 1954  
2,706,677 Duncan et al. ----- Apr. 19, 1955  
2,784,067 Duncan et al. ----- Mar. 5, 1957

UNITED STATES PATENT OFFICE  
CERTIFICATE OF CORRECTION

Patent No. 2,920,944

January 12, 1960

Troy L. Cantrell et al.

It is hereby certified that error appears in the printed specification of the above numbered patent requiring correction and that the said Letters Patent should read as corrected below.

Column 6, line 16, after "acid" and before the period insert --, said minor amount being about 0.1 to about 0.001 per cent by weight of the composition --.

Signed and sealed this 21st day of June 1960.

(SEAL)

Attest:

KARL H. AXLINE

Attesting Officer

ROBERT C. WATSON  
Commissioner of Patents